

**1**

3,684,507

**DATA STORAGE SYSTEMS**Ronald Francis, Arlington, Mass., assignor to Itek  
Corporation, Lexington, Mass.

No Drawing. Continuation of abandoned application Ser. No. 463,037, June 10, 1965. This application Aug. 12, 1968, Ser. No. 755,015

Int. Cl. G03c 5/04, 5/24

U.S. Cl. 96—27

20 Claims

**ABSTRACT OF THE DISCLOSURE**

A data storage medium comprising a support and a radiation sensitive titanium dioxide, the titanium dioxide having been heated at an elevated temperature and for a time period sufficient to increase the photographic speed thereof. Preferably, the titanium dioxide has been heated to a temperature of at least 200° C. for a time period of at least 0.5 hour. This copy medium can then be exposed to establish an image pattern and if desired, contacted with suitable image forming material to establish a permanent image.

Preferred image forming materials comprise a liquid redox system such as a solution of metal ions.

This application is a continuation of application Ser. No. 463,037, filed June 10, 1965, and now abandoned.

Data or image storage media comprising radiation sensitive titanium dioxide are described in detail in U.S. Pats. 3,152,903; 3,152,904; 3,052,541; French Pats. 345-206 and 1,245,215, and in commonly owned copending U.S. patent application Ser. No. 199,211, filed May 14, 1962, by Elliot Berman et al. and now abandoned. In the aforesaid U.S. patent application, radiation sensitive titanium dioxide functions as the photosensitive component of the media. As described in said application, exposure of said media to a pattern of radiant energy results in the storage of a reversible image pattern of radiant energy results in the storage of a reversible image pattern therein. The reversible image pattern exists for a limited time during which said pattern can be converted to an irreversible form and read out visually by contacting said pattern with chemical redox systems. In the aforesaid U.S. and French patents, the radiation sensitive titanium dioxide apparently functions as an accelerator or as an auxiliary photosensitive component of the media described. In view of the many image storage systems having media comprising radiation sensitive titanium dioxide, improved media of this type which are especially advantageous in said systems would be indeed a notable contribution to the art.

A principal object of the present invention is to provide improved data storage systems.

Another object of the present invention is to provide improved data or image storage systems involving media comprising titanium dioxide as a component thereof.

Another, more specific object of the present invention is to provide an improved image storage system wherein said image is stored in reversible form in media comprising radiation sensitive titanium dioxide.

Still another object of the present invention is to provide an improved storage system wherein the image pattern obtained upon exposure of the media can be converted to an irreversible form at a preselected time or space remote from that at which said exposure occurred.

Still another specific object of the present invention is to provide an image storage system wherein the image pattern obtained upon exposure of the media can be selectively erased from said media or altered while stored in 70 said media, such as by addition thereto.

Another object of the present invention is to provide

**2**

a method for selectively adjusting the principal photographic properties of image storage media comprising radiation sensitive metal oxides and for producing image storage media of predetermined photographic properties.

5 Still other objects and advantages of the present invention will in part be obvious to those skilled in the art or will in part appear hereinafter.

Broadly, the abovementioned objects and advantages are realized in accordance with the practice of the present invention by including in data or image storage media of the type described, a particular titanium dioxide which has been aftertreated at elevated temperatures in an oxidizing atmosphere. More precisely, I have found that surprisingly improved photographic properties of such data storage media can be obtained by including therein a heat treated, radiation sensitive titanium dioxide which had an initial particle size substantially less than about 1 micron and a nitrogen surface area of less than about 60 square meters per gram prior to the heat treatment thereof.

10 20 The best balance of improved properties are obtained in media comprising a heat treated titanium dioxide which was produced by the high temperature pyrolysis of titanium halides and, as produced, had an initial average particle diameter of less than about 0.2 micron and an initial

15 25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000

5 10 15 20 25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000

5 10 15 20 25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000

5 10 15 20 25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000

5 10 15 20 25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000

5 10 15 20 25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000

transparent or translucent when cured, such as a copolymer of styrene and butadiene, more commonly known as "Pliolite," and polyamide, more commonly known as "Zytel 61." Representative preferred transparent or translucent substrates include those comprising polyethylene terephthalate, polyesters, cellulose acetate, and the like.

Details of my invention and of the benefits to be obtained therefrom will be better understood by reference to the following examples which describe methods of practicing same. The following examples are to be considered as illustrative in nature and in no way are they to be construed so as to limit my invention beyond those limitations expressly set forth in the present specification or in the claims which appear hereinafter.

#### EXAMPLE 1

Sixteen parts by weight of a finely divided titanium dioxide—"Cabot P-25"—having an average particle size of about 0.03 micron and an initial surface area of about 40 square meters per gram were dispersed in about 75 parts by weight of water in which 0.32 part by weight of sodium hexametaphosphate had been added as a dispersing agent. The pigment was added with stirring, and the mixture was thoroughly agitated to disperse the titanium dioxide uniformly therethrough.

About 8.5 parts by weight of 47 percent "Rhoplex," aqueous polyacrylate latex, were next combined with the dispersion containing the particulate titanium dioxide. The mixture, which was thoroughly stirred, thus contained about 4 parts of acrylate solids by dry weight, so that the weight ratio of  $TiO_2$  to binder solids was 4 to 1. The resulting mixture was coated on a transparent substrate. The coating weight of said photosensitive medium was about six pounds per 3,000 square feet.

The medium was then exposed to a standard xenon flash source in a Mark VI EG&G sensitometer for about  $10^{-3}$  seconds.

The medium so exposed was then immersed in a saturated methanolic solution of silver nitrate and subsequently in an amplification solution comprising about 30 grams of phenidone and 30 grams of citric acid in about one liter of methanol.

The photographic properties of the above medium were determined in accordance with a standard sensitometry technique as described in detail in a publication entitled "Sensitometry and Grading of Photographic Papers" published by the American Standards Association in 1953. The following data were obtained:

TABLE 1.—PHOTOGRAPHIC PROPERTIES

|                               |      |
|-------------------------------|------|
| Gamma (contrast) -----        | 1.1  |
| Speed -----                   | 14   |
| Maximum optical density ----- | 1.1  |
| Fog level -----               | 0.08 |

#### EXAMPLE 2

A sample of the "Cabot P-25" of Example 1 was heated in air at a temperature of 650° C. for about 2 hours.

After heat treatment, the nitrogen surface area was 65 square meters per gram while the average particle diameter appeared to be relatively unaffected.

Thereafter the titanium dioxide so heat treated was included in an image storage medium and an image stored in and retrieved therefrom in accordance with the procedure set forth in Example 1.

The photographic properties of the medium were determined as in Example 1 and the following data were obtained:

TABLE 2.—PHOTOGRAPHIC PROPERTIES

|                               |      |
|-------------------------------|------|
| Gamma (contrast) -----        | 0.98 |
| Speed -----                   | 165  |
| Maximum optical density ----- | 1.1  |
| Fog level -----               | 0.09 |

#### EXAMPLE 3

Substantially the same procedure as set forth in Example 1 was followed, but, instead of "Cabot P-25," a precipitated titanium dioxide was included as the photosensitive component of the medium. The precipitated titanium dioxide had an initial average particle size of about 0.2 micron and an initial nitrogen surface area of about 10 square meters per gram.

The photographic properties of the medium were determined and the following data were obtained:

TABLE 3.—PHOTOGRAPHIC PROPERTIES

|                               |      |
|-------------------------------|------|
| Gamma (contrast) -----        | 0.76 |
| Speed -----                   | 7.0  |
| Maximum optical density ----- | 0.80 |
| Fog level -----               | 0.08 |

#### EXAMPLE 4

Substantially the same procedure as set forth in Example 2 was followed, but, instead of "Cabot P-25," the precipitated titanium dioxide of Example 3 was heated in air at a temperature of 400° C. for about 3 hours.

The photographic properties of the image storage medium comprising the precipitated titanium dioxide so heat treated were determined and the following data were obtained:

TABLE 4.—PHOTOGRAPHIC PROPERTIES

|                               |      |
|-------------------------------|------|
| Gamma (contrast) -----        | 0.78 |
| Speed -----                   | 20   |
| Maximum optical density ----- | 0.84 |
| Fog level -----               | 0.07 |

#### EXAMPLE 5

Substantially the same procedure as set forth in Example 1 was followed, but, instead of "Cabot P-25," "Cabot P-110" was included as the photosensitive component of the medium. "Cabot P-110" is a titanium dioxide produced by the pyrolysis of titanium halides and has an initial average particle size of about 0.1 micron and an initial nitrogen surface area of about 20 square meters per gram.

The photographic properties of the medium were determined and the following data were obtained:

TABLE 5.—PHOTOGRAPHIC PROPERTIES

|                               |      |
|-------------------------------|------|
| Gamma (contrast) -----        | 0.73 |
| Speed -----                   | 10   |
| Maximum optical density ----- | 1.1  |
| Fog level -----               | 0.08 |

#### EXAMPLE 6

Substantially the same procedure as set forth in Example 2 was followed, but, instead of "Cabot P-25," "Cabot P-110" was heated in air at a temperature of 500° C. for about 5 hours.

The photographic properties of the image storage medium comprising the "Cabot P-110" so heat treated were determined and the following data were obtained:

TABLE 6.—PHOTOGRAPHIC PROPERTIES

|                               |      |
|-------------------------------|------|
| Gamma (contrast) -----        | 0.65 |
| Speed -----                   | 32   |
| Maximum optical density ----- | 1.0  |
| Fog level -----               | 0.07 |

Examples 1 through 6 dramatically illustrate the improvements obtained in image storage media produced in accordance with the practice of my invention. It is to be understood that any of the heat treated titanium dioxides or mixtures thereof can be combined with non-heat treated titanium dioxides to produce image storage media of predetermined photographic properties. Accordingly, the practice of my invention enables one to selectively prepare image storage media of a wide range of predetermined photographic properties.

## EXAMPLE 7

A medium prepared in accordance with the procedure set forth in Example 1 was immersed in a saturated solution of silver nitrate in methanol prior to the exposure thereof.

After drying, the medium was exposed to the standard source.

After exposure, the medium was then developed in a methanolic solution comprising 10 grams of phenidone and 80 grams of citric acid per liter.

The photographic properties of the medium were determined and the following data were obtained:

TABLE 7.—PHOTOGRAPHIC PROPERTIES

|                               |      |
|-------------------------------|------|
| Gamma (contrast) -----        | 1.0  |
| Speed -----                   | 35   |
| Maximum optical density ----- | 1.5  |
| Fog level -----               | 0.11 |

## EXAMPLE 8

A medium prepared in accordance with the procedure set forth in Example 2 was immersed in a saturated solution of silver nitrate in methanol prior to the exposure thereof.

After drying, the medium was exposed to the standard source and developed in accordance with the procedure of Example 7.

The photographic properties of the medium were determined and the following data obtained:

TABLE 8.—PHOTOGRAPHIC PROPERTIES

|                               |      |
|-------------------------------|------|
| Gamma (contrast) -----        | 1.0  |
| Speed -----                   | 190  |
| Maximum optical density ----- | 1.5  |
| Fog level -----               | 0.10 |

Examples 7 and 8 illustrate the improvements realized when media comprising other photosensitive components include the heat treated titanium dioxides of the present invention.

Many modifications of the details involved in the above examples offered for the purpose of illustrating my invention may be utilized in the practice thereof without departing from the spirit and scope of the invention defined in the appended claims.

Having described my invention and methods of practicing same together with preferred embodiments thereof, what I declare as new and desire to secure by U.S. Letters Patents is as follows:

1. In a data storage medium comprising a support and a radiation sensitive titanium dioxide dispersed in a binder, the improvement wherein the titanium dioxide is a titanium dioxide which is heated in an oxidizing atmosphere at an elevated temperature of at least about 200° C. for a time period of at least about 0.5 hour and which had an initial average particle diameter no greater than about one micron and a nitrogen surface area of less than about 60 square meters per gram prior to this heating, the titanium dioxide which is subjected to this heating being such that the photographic speed of the titanium dioxide will be improved by such heating when subsequently utilized in a photographic process involving exposing a copy medium comprising the titanium dioxide and forming a permanent image by contacting with image-forming materials which undergo an oxidation-reduction type reaction.

2. The medium of claim 1 wherein the titanium dioxide is heated in an oxidizing atmosphere at a temperature of at least about 400° C. for a time period of at least about 0.5 hour.

3. The medium of claim 1 wherein the titanium dioxide is heated at a temperature between about 400° C. to about 650° for from about 2 hours to about 5 hours.

4. The medium of claim 1 wherein the titanium dioxide had an initial average particle size no greater than about 0.2 micron.

5. The medium of claim 1 wherein the titanium dioxide to be heated is produced by the high temperature pyrolysis of titanium halides.

6. The medium of claim 1 wherein the titanium dioxide to be heated is produced by the high temperature pyrolysis of titanium halides and had an initial average particle diameter of about 0.03 micron and an initial nitrogen surface area of about 40 square meters per gram.

7. In the process wherein a data storage medium comprising a support and a photosensitive titanium dioxide dispersed in a binder is exposed to establish an image pattern, the improvement wherein the titanium dioxide is a titanium dioxide which is heated in an oxidizing atmosphere at a temperature of at least about 200° C. for a period of time of at least about 0.5 hour and which titanium dioxide had an initial average particle diameter no greater than about one micron and a nitrogen surface area of less than about 60 square meters per gram prior to this heating, the titanium dioxide which is subjected to

this heating being such that the photographic speed of the titanium dioxide will be improved by such heating when subsequently utilized in a photographic process involving exposing a copy medium comprising the titanium dioxide and forming a permanent image by contacting with image-forming materials which undergo an oxidation-reduction type reaction.

8. The process of claim 7 wherein the titanium dioxide is heated in an oxidizing atmosphere at a temperature of at least about 400° C.

9. The process of claim 8 wherein said titanium dioxide is heated at a temperature between about 400° C. to about 650° C. for from about 2 to about 5 hours.

10. The process of claim 8 wherein said titanium dioxide had an initial average particle size no greater than about 0.2 micron.

11. The process of claim 8 wherein said titanium dioxide to be heated is produced by the high temperature pyrolysis of titanium halides.

12. The process of claim 11 wherein said titanium dioxide is produced by the high temperature pyrolysis of titanium halides and had an initial average particle diameter of about 0.03 micron and an initial nitrogen surface area of about 40 square meters per gram prior to this heating.

13. A process for producing an image comprising the steps of:

(a) exposing imagewise a data storage medium comprising a support and a radiation sensitive titanium dioxide dispersed in a binder, which titanium dioxide is heated in an oxidizing atmosphere at elevated temperatures of at least about 200° C. and for a period of time of at least about 0.5 hour and for a period of time sufficient to increase the photographic speed of the medium and which had an initial particle diameter of no greater than about 0.2 micron and a nitrogen surface area of less than about 60 square meters per gram, the titanium dioxide which is subjected to this heating being such that the photographic speed of the titanium dioxide will be improved by such heating when subsequently utilized in a photographic process involving exposing a copy medium comprising the titanium dioxide and forming a permanent image by contacting with image-forming materials which undergo an oxidation-reduction type reaction; and

(b) contacting the medium with image-forming materials which undergo an oxidation-reduction type reaction to form a permanent image thereon.

14. The process of claim 13 wherein the titanium dioxide was heated in an oxidizing atmosphere at a temperature of at least about 400° C.

15. The process of claim 14 wherein the titanium dioxide to be heated was produced by the high temperature pyrolysis of titanium halides.

16. The process of claim 14 wherein the titanium dioxide which was heated to increase the photographic speed of the data storage medium is used in combination with at least one other photosensitive material.

17. The process of claim 14 wherein the data storage medium includes image-forming materials at the time of exposure thereof.

18. In a data storage medium comprising a radiation sensitive titanium dioxide dispersed in a binder, image-forming materials which undergo an oxidation-reduction type reaction, and a support therefor, the improvement wherein the titanium dioxide is a titanium dioxide which had an initial average particle diameter no greater than about one micron and a nitrogen surface area of less than about 60 square meters per gram and which was heated in an oxidizing atmosphere at an elevated temperature of at least about 200° C. and for a time period of at least about 0.5 hour and sufficient to increase the photographic speed thereof, the titanium dioxide which is subjected to this heating being such that the photographic speed of the titanium dioxide will be improved by such heating when subsequently utilized in a photographic process involving exposing a copy medium comprising the titanium dioxide and forming a permanent image by contacting

with image-forming materials which undergo an oxidation-reduction type reaction.

19. A medium as in claim 18 wherein the image forming materials comprise a source of metal ions.

5 20. A medium as in claim 18 wherein the image forming materials comprise a source of silver ions.

#### References Cited

##### UNITED STATES PATENTS

|    |           |         |                       |        |
|----|-----------|---------|-----------------------|--------|
| 10 | 3,198,632 | 8/1965  | Kimble et al. _____   | 96—1.8 |
|    | 3,311,452 | 3/1967  | Goodgame et al. _____ | 23—202 |
|    | 3,317,321 | 5/1967  | Chopoorian _____      | 96—88  |
|    | 3,380,823 | 4/1968  | Gold _____            | 96—27  |
| 15 | 3,397,982 | 8/1968  | Lane _____            | 96—1.5 |
|    | 3,409,429 | 11/1968 | Ekman et al. _____    | 96—27  |
|    | 3,424,582 | 1/1969  | Berman et al. _____   | 96—48  |

CHARLES E. VAN HORN, Primary Examiner

20 U.S. Cl. X.R.

96—1.5, 48 PD, 67, 88; 117—1.7; 106—300; 23—202 R; 252—501